

Sept. 3, 1968

R. GROTH

3,400,288

SODIUM VAPOR DISCHARGE LAMP WITH INFRARED REFLECTING COATING

Filed Nov. 8, 1966



FIG.1



FIG.2

INVENTOR.  
ROLF GROTH

BY

*Frank R. Sinfani*  
AGENT

3,400,288  
SODIUM VAPOR DISCHARGE LAMP WITH  
INFRARED REFLECTING COATINGRolf Groth, Aachen, Germany, assignor to North American  
Philips Co., Inc., New York, N.Y., a corporation  
of Delaware

Filed Nov. 8, 1966, Ser. No. 592,859

Claims priority, application Germany, Nov. 13, 1965  
N 27,625  
4 Claims. (Cl. 313—47)

## ABSTRACT OF THE DISCLOSURE

A sodium vapor lamp provided with a heat-reflective  
light-transmissible coating of doped  $In_2O_3$  on the inner  
wall of the outer envelope.The invention relates to a sodium vapor discharge  
lamp having a transparent envelope which, preferably  
on the side facing the discharge tube, is coated with a  
layer which transmits visible light and reflects infrared  
radiation.The luminous efficiency of sodium vapor discharge  
lamps can be improved by using such selectively reflecting  
layers. The use of thin metal layers as well as  
of tin dioxide layers for this purpose is already known.With gold layers of a thickness of approximately 150  
A. it is possible, for example, to increase the luminous  
efficiency of a sodium vapor discharge lamp by approxi-  
mately 20% as compared with a lamp without an infrared  
reflecting layer. This higher luminous efficiency in  
lumens per watt is obtained only, however, if the  
electric power supplied to the lamp is reduced to ap-  
proximately one fourth as compared with a sodium vapor  
lamp without a gold layer. As a result of this, the luminous  
flux decreases to approximately one third. This decrease  
of the luminous flux has two causes. First, due to the  
improved heat insulation a smaller current is sufficient  
to reach the optimum operating temperature of the dis-  
charge tube; consequently, however, the excitation density,  
that is to say, the amount of electrons which excite the  
Na atoms is accordingly smaller. In addition, losses of  
light occur as a result of absorption and reflection of  
the gold filter.However, an improvement in this respect is obtained  
if a tin dioxide layer is used instead of a gold layer.Although the reflecting power of tin dioxide for waves  
exceeding 4  $\mu m$ ., which supply the essential part for the  
thermal radiation of sodium vapor discharge lamps is  
smaller than that of a gold layer, the permeability of the  
tin dioxide filter nevertheless is so much higher that both the quantity of light produced and the luminous  
efficiency are larger than in a lamp with a gold layer.As is known, the selective reflective behavior of highly-doped semiconductor layers in the infrared spectrum is  
obtained by the variation of the susceptibility of the  
crystal lattice, as a result of a high concentration of  
free charge carriers. If a high reflecting power in the  
infrared region is to be achieved, the concentration of  
the free charge carriers on the basis of theoretical  
considerations, must exceed  $10^{20}/cm^3$  and the mobility of  
the said carriers must be as large as possible.The manufacture of tin metal oxide on glass supports  
by thermal decomposition of suitable metal compounds  
has been known for a long time. Usually the so-called  
atomization method is used. In this method, the metal  
compound is atomized together with a suitable solvent  
by means of a nozzle and this mixture is blown against  
the hot glass support in the form of a fine mist, the  
conversion into metal oxide then occurring.A drawback of these known methods is that the tin  
dioxide layers manufactured in this manner are difficult  
to reproduce as regards their optical and electrical properties.  
For example, the reflecting power in the infrared  
spectrum ( $\lambda=8 \mu m$ ) fluctuates between 45 and 80%.  
For the mobility of the free-charge carriers values be-  
tween 3 and 15  $cm^2/volt\cdot sec$ . are found. The electrical  
optical properties in tin dioxide layers are so poorly  
reproducible because they strongly depend upon the tem-  
perature at which the oxide is formed.In the normal spraying methods, the glass plates are  
cooled considerably during spraying as a result of the  
accompanying cold air. When the thickness of the layer  
increases the specific conductivity therefore becomes  
worse. With such non-homogeneous layers no reproducible  
results, that is to say poor reflection filters are to be  
expected of course. Therefore, in the manufacture of  
tin dioxide layers several short-lasting spraying operations  
are carried out in order that the supporting plates  
are not cooled considerably and can be heated again dur-  
ing the pauses in the spraying operations, or the atom-  
ized mixture must be heated beforehand, or both meas-  
ures must be combined.It has now been found that these drawbacks can be  
considerably mitigated in the manufacture of heat re-  
flection filters constituted of indium oxide. In addition,  
the indium oxide layers show a higher reflecting power  
in the infrared spectrum and a higher permeability for  
sodium light than tin dioxide ( $SnO_2$ ).According to the invention, the coating layer substan-  
tially consists of doped indium oxide ( $In_2O_3$ ).It has been found, that in contrast with the manufac-  
ture of layers from tin dioxide it is not necessary for  
this purpose to take particular measures to obtain re-  
producible layers having good reflecting powers.It has been found that the conductivity and the in-  
frared reflecting power of indium oxide layers at tem-  
peratures of manufacture above 400° C. do not depend  
upon the manufacturing temperature. This is a decisive  
advantage of the indium oxide layers as compared with  
tin oxide layers in which the conductivity and the re-  
flecting power vary considerably with the temperature of  
manufacture.The invention will now be described with reference to  
the accompanying drawing, in which:FIG. 1 shows reflection curves of prior art and re-  
flective coatings according to the invention.FIG. 2 shows a sodium vapor lamp according to the in-  
vention.FIG. 1 shows the infrared reflecting power of two  
 $In_2O_3$  layers (curves 1 and 2) and of two  $SnO_2$  layers  
(curves 3 and 4) of the same thickness. The  $In_2O_3$  layers  
were manufactured at temperatures of 500° C. (curve 1)  
and 400° C. (curve 2) of the supporting plate. The  $SnO_2$   
layers were likewise manufactured at 500° C. (curve 3)  
and 400° C. (curve 4).In manufacturing the layers, a solution of an indium  
compound was atomized through a nozzle and the atom-  
ized mixture blown in a cold condition against a hot glass  
plate. The temperature of the glass plate was chosen to  
be higher than 400° C. and preferably was between 400°  
C. and the softening temperatures of the glass. When  
using aqueous solutions only dull layers are usually ob-  
tained which are of no interest as filters. Entirely bright  
layers are obtained on the contrary if organic solvents,  
for example, butyl acetate and butanol, are used. Indium  
compounds, which may be used, are, for example,  $InCl_3$   
and the other halides of indium.For a high reflecting power in the infrared spectrum,  
it is necessary that the conductivity of the layers of this  
type be as high as possible. It should be at least larger  
than approximately  $2 \times 10^3$  ohms $^{-1}$ —cm. $^{-1}$ . If only in-

dium compounds are used these conductivities cannot be obtained. For example, the conductivity when  $\text{InCl}_3$  alone was used, reached values only up to  $2 \times 10^2 \text{ ohms}^{-1} \text{ cm.}^{-1}$ . The conductivity, and consequently the infrared reflecting power, can be increased considerably if particular dopings are added to the starting solution. The best results were obtained with Sn-doping (in the form of  $\text{SnCl}_4$ ) and F-doping (in the form of a soluble fluorine compound, for example HF). Conductivities were obtained, for example up to  $42 \times 10^3 \text{ ohms}^{-1} \text{ cm.}^{-1}$ .

Investigations into layers of different thicknesses have proved that with layer thicknesses above  $0.5 \mu\text{m}$ . usually dullness occurs as a result of which the permeability for sodium light is reduced. Layers having a thickness of below approximately  $0.5 \mu\text{m}$ . are entirely absorption-free for sodium light and its permeability is only modified by interference effects. Therefore, the layer thickness should be chosen to be such that for sodium light a permeability maximum occurs. However, it was found that in the case of thin layers below approximately  $0.20 \mu\text{m}$ . the reflecting power decreased considerably. Particularly good results were obtained with layer thicknesses of approximately  $0.31 \mu\text{m}$ . and approximately  $0.46 \mu\text{m}$ . respectively. In both layer thicknesses a permeability of 91% is obtained for sodium light ( $\lambda$  approximately  $0.59 \mu\text{m}$ ) (permeability of the glass plate without layer approximately 91–92%).

The reflecting power in the infrared spectrum of the layer of  $0.31 \mu\text{m}$ . was substantially of the same value as that of the  $0.46 \mu\text{m}$ . layer. Both layers reached a reflecting power of approximately 90% and  $10 \mu\text{m}$ . A tin dioxide layer of  $0.32 \mu\text{m}$ . thickness manufactured under optimum conditions had a permeability of 89% for sodium light and an infrared reflecting power of 80%.

The invention also will be described in greater detail with reference to the following examples and the table.

#### Example

Layers were manufactured by spraying a solution of  $\text{InCl}_3$  in butyl acetate, containing 40 gm. of  $\text{InCl}_3$  per liter of butyl acetate and a respective quantity of  $\text{SnCl}_4$  as shown in Table 1. The layer thickness was  $0.32 \mu\text{m}$ . The table shows the surface resistance  $R_s$  in  $\text{ohms}^2$ , the electrical conductivity  $\lambda$  in  $\Omega^{-1} \cdot \text{cm.}^{-1}$   $\text{ohms}^{-1} \text{ cm.}^{-1}$ , the concentration of the free charge carriers  $N$  (per  $\text{cm.}^3$ ) and their Hall-mobility,  $\mu$  in  $\text{cm.}^2/\text{volt}\cdot\text{sec.}$  in accordance with the Sn-addition which is stated in atomic percent relative to In and was calculated from the added quantity of  $\text{SnCl}_4$ .

TABLE 1

| At. percent Sn | $R_s$ ( $\Omega$ ) | $\lambda$ ( $\Omega^{-1} \cdot \text{cm.}^{-1}$ ) | $N$ ( $\text{cm.}^{-3}$ ) | $\mu$ $\text{cm.}^2/\text{volt sec.}$ |
|----------------|--------------------|---------------------------------------------------|---------------------------|---------------------------------------|
| 0.03           | 115.1              | $2.62 \times 10^2$                                | $2.36 \times 10^{19}$     | 71.9                                  |
| 0.3            | 41.0               | $7.64 \times 10^2$                                | $4.2 \times 10^{19}$      | 71.4                                  |
| 0.7            | 14.8               | $2.11 \times 10^3$                                | $1.97 \times 10^{20}$     | 66.8                                  |
| 1.5            | 9.54               | $3.02 \times 10^3$                                | $3.96 \times 10^{20}$     | 48.2                                  |
| 1.8            | 9.00               | $3.48 \times 10^3$                                | $4.95 \times 10^{20}$     | 43.8                                  |
| 2.3            | 7.34               | $4.25 \times 10^3$                                | $5.70 \times 10^{20}$     | 46.6                                  |
| 2.8            | 8.69               | $3.68 \times 10^3$                                | $5.98 \times 10^{20}$     | 38.5                                  |
| 3.7            | 9.70               | $3.23 \times 10^3$                                | $5.76 \times 10^{20}$     | 35.1                                  |
| 5.5            | 8.55               | $3.65 \times 10^3$                                | $6.57 \times 10^{20}$     | 34.8                                  |

It may be seen from the table that the surface resistance  $R_s$  decreases with an increasing Sn-addition and reaches a minimum at approximately 2.3 atomic percent. In addition, it may be seen that the concentration of the free charge carriers  $N$  increases when the Sn-addition increases. However, with large additions, the mobility again

decreases so that maximum conductivity is reached with approximately 2.3 atomic percent Sn-addition. Additions in this range consequently are at an optimum for optimum conductivity and high infrared reflecting power. In the case of a doping with fluorine, optimum results are obtained with additions of approximately 2 atomic percent relative to indium.

5 The discharge tube 1 (FIG. 2) is surrounded by an evacuated glass outer envelope 4 provided with lamp sockets 2 and 3. The discharge tube includes two electrodes 5 and 6 and contains, in addition to the required quantity of sodium metal, a neon gas filling with a slight addition of argon.

10 Three lamps having the same geometric proportions on the inside were compared with one another. In lamp I, the outer envelope 4 was coated on the inside with a gold layer,  $0.015 \mu\text{m}$ . thick. In lamp II the outer envelope 4 was coated on the inside with a tin dioxide layer,  $0.32 \mu\text{m}$ . thick. This layer contained approximately 2 atomic percent of F relative to the quantity of tin as a dopant. In lamp III the outer envelope 4 was coated on the inside with an indium oxide layer according to the invention  $0.31 \mu\text{m}$ . thick. The layer contained 2.3 atomic percent of Sn relative to the quantity of indium as a dopant.

15 The measured results as shown in Table 2 were obtained:

TABLE 2

|                                         | I     | II     | III    |
|-----------------------------------------|-------|--------|--------|
| Consumed electric power (watts) .....   | 70    | 128    | 85     |
| Luminous flux (lumens) .....            | 8,750 | 16,900 | 14,100 |
| Luminous efficiency (lumens/watt) ..... | 125   | 132    | 166    |

20 While the invention has been described with reference to particular embodiments and applications thereof, other modifications will be obvious to those skilled in this art without departing from the spirit and scope thereof as defined in the appended claims.

25 What is claimed is:

1. A sodium vapor discharge lamp comprising an envelope permeable to visible radiation surrounding a discharge space in which visible light is produced by an electrical discharge through an ionizable medium containing sodium ions, an infrared radiation reflective coating on the inner wall of said envelope permeable to visible light, 30 said layer consisting essentially of indium oxide ( $\text{In}_2\text{O}_3$ ) doped with an amount of an element taken from the group consisting of tin and fluorine at which the surface resistivity of said layer is a minimum.

2. A sodium vapor discharge lamp as claimed in claim 1 in which the coating layer contains between 1.5 and 5.5 atomic percent of tin relative to the quantity of In.

3. A sodium vapor discharge lamp as claimed in claim 1 in which the coating layer contains approximately 2.3 atomic percent of tin relative to the quantity of In.

4. A sodium vapor discharge lamp as claimed in claim 1 in which the coating layer contains approximately 2 atomic percent of fluorine relative to the quantity of In.

#### References Cited

#### UNITED STATES PATENTS

- 2,564,708 8/1951 Mochel ..... 117—33.3  
 3,221,198 11/1965 Van Der Wal et al. .... 313—112  
 3,295,002 12/1966 Amans ..... 313—108

60 65 DAVID J. GALVIN, Primary Examiner.